

Oct. 4, 1932.

C. R. NOLLER

1,880,466

PROCESS OF MAKING CELLULOSE ACETATE WITH VAPORIZED ACETYLATING AGENTS

Filed Feb. 2, 1928



Inventor,  
Carl R. Noller,

By R. L. Stinchfield

Attorney

## UNITED STATES PATENT OFFICE

CARL R. NOLLER, OF ROCHESTER, NEW YORK, ASSIGNOR TO EASTMAN KODAK COMPANY, OF ROCHESTER, NEW YORK, A CORPORATION OF NEW YORK

## PROCESS OF MAKING CELLULOSE ACETATE WITH VAPORIZED ACETYLATING AGENTS

Application filed February 2, 1928. Serial No. 251,297.

This invention relates to processes of making cellulose acetate using vaporized acetylating agents. One object of the invention is to provide a process of this nature in which the desired acetylation of cellulosic materials can be effected within a useful time, and yet the product will not be seriously degraded nor contaminated with unacetylated fibers. Other objects will hereinafter appear.

In the accompanying drawing the single figure is a diagrammatic sectional view on an exaggerated scale of one type of apparatus in which my process may be carried out.

In U. S. Patent No. 1,030,311, Koetschet and Theumann, June 25, 1912 "Acetylation of cellulosic materials" there is disclosed a process of making cellulose acetate in which acetic anhydrid vapors are passed through cotton from a vaporizer to a condenser. The system may be under sub-atmospheric pressure in order to assist the boiling of the acetic anhydrid in the vaporizer. When a molecule of acetic anhydrid reacts with a molecule of cellulose, there is liberated a molecule of acetic acid. This acid has a boiling point always less than that of acetic anhydrid at the same pressure. Consequently, any acetic acid present in the cotton initially, or formed during the reaction by the process of said patent, will be immediately carried by the stream of acetic anhydrid vapor into the condenser and liquefied there.

I have found that the reaction may be regulated to obtain the desired results mentioned above by retaining at least part of the vapor of acetic acid, liberated by the reaction, in contact with the cellulosic material which is being treated. Since enough of this acid is rapidly liberated at the start of the reaction to saturate the reaction space with acetic acid vapor, and to keep it saturated until the material is acetylated, practically the entire process is carried out by a mixture of saturated vapors of acetic anhydrid and acetic acid. Preferably the air is eliminated from the reaction space, say by evacuating it, prior to conducting the reaction. Of course, the cellulosic material is mixed with one of the known agents that promotes acetylation. In the preferred form of my inven-

tion I do not employ a stream of the mixed anhydrid and acid vapors, but merely heat the cellulosic material in a closed vessel containing an open body or pool of acetic anhydrid. The latter may be in a container above the cellulose to be treated, and the acetic anhydrid vapors can diffuse over the edges of the container down into the cellulosic material. The product, which is obtained in an undissolved state, retains the original fibrous or other form of the raw material, and is soluble in chloroform when the reaction is carried through to completion.

The cellulosic material may be any of those heretofore used in making cellulose acetate by the use of acetic anhydrid in liquid form, such as purified cotton wool, tissue paper prepared from clean cotton fibers, surgical cotton wool, and even bleached sulfite wood pulp, or cotton linters which have been given a mild alkaline boil and bleaching treatment. Likewise, I can acetylate cellulosic compounds which have been partially esterified or etherified, such as lower cellulose nitrates, lower cellulose acetates, and lower cellulose ethers.

My process may be carried out with the aid of most of the catalysts or agents for promoting acetylation which have been used in the prior art with liquid acetic anhydrid. I prefer, however, to use liquid agents with which the cellulosic material may be readily impregnated, said liquids being of low volatility relative to acetic anhydrid. Because of their cheapness, sulfuric acid and para-toluene sulfonic acid serve as excellent examples.

I shall now describe several examples of my invention, but it will be understood that the latter is not limited to the details thus given, except as indicated in the appended claims. In a closed vessel there is placed 2 parts by weight of air-dried purified cotton, previously impregnated with .23% of its weight of sulfuric acid. In an open container in the same closed vessel there is placed 20 parts by weight of acetic anhydrid. From the closed vessel the air is exhausted until a relatively high vacuum is reached, say a pressure of 10 millimeters of mercury. The

vessel and its contents are then heated to 60° to 65° C. and kept at that temperature until the reaction has proceeded to the desired point. When the contents are heated, as mentioned above, the vapors of acetic anhydrid rapidly evolve in the closed vessel and come in contact with all of the exposed surface of the cotton containing the catalyst. The reaction then starts and acetic acid is formed, which vaporizes and mingles with the acetic anhydrid vapors throughout the closed vessel, thus remaining in contact with the cotton throughout the rest and main part of the reaction. Moreover, the acetic acid vapor rapidly reaches saturation and remains saturated throughout the reaction. The end point of the reaction is found by taking samples from time to time and testing their solubility in chloroform, or in a mixture of equal parts of chloroform and alcohol. Under the conditions just given, full solubility has been obtained, together with an acetyl content of 43.9% in as short a time as 39 hours.

In still another example of my invention, 100 parts by weight of air-dried purified cotton is impregnated with 1% of its weight of paratoluene sulfonic acid. This is placed in a vessel containing, above it, an open receptacle in which there is 280 parts by weight of acetic anhydrid (95% strength). The vessel is carefully sealed and the air removed by a preliminary evacuation down to about a pressure of 10 millimeters of mercury. The interior of the vessel, including the cotton and the acetic anhydrid, is kept at 60° to 65° C., until the desired solubility and acetyl content is reached in the product. Under such conditions there is obtained fully chloroform-soluble fibers after about 72 hours. It is one of the features of this process that it is economical of anhydrid and only slightly more than the theoretical amount required for the acetylation is consumed. I prefer to have the receptacle containing the acetic anhydrid above the cotton in the closed vessel, rather than below it, because a much more even diffusion of anhydrid is obtained, with a consequent uniform acetylation throughout the cotton. Where the anhydrid is below the cotton, the lower layers of the latter become completely acetylated before the portions at the top.

Referring to the accompanying drawing, 1 indicates a closed vessel composed of or lined with any suitable material which is resistant to the vapors of acetic anhydrid and acetic acid under the conditions stated above. This vessel may be heated in any suitable manner, say by a jacket 2 through which there is circulated a suitable heating fluid, which enters through pipe 3 controlled by valve 31 and leaves through pipe 4 controlled by valve 41. The cover 5 of the vessel 1 is detachably held in gas-tight contact with the

rest of vessel 1 by any of the usual means, such as the swinging bolts 6. Leading from the top of cover 5 is a pipe 7, controlled by valve 71, which leads to the vacuum apparatus. Within the vessel 1 in the upper part thereof is a support 8 upon which there is an open receptacle 9 in which there is a body of liquid acetic anhydrid 10. Below the receptacle 9 there is located the cellulosic material, such as cotton 11. The vapors rising from anhydrid 10 diffuse down and through the cotton 11 and become mingled with the vapors of acetic acid liberated in the reaction, as described above in connection with the examples.

Having thus described my invention, what I claim as new and desire to secure by Letters Patent is:

1. In the process of making cellulose acetate, placing cellulosic fibers, impregnated with an agent which promotes acetylation, in part of an enclosed space, placing an open body of liquid acetic anhydrid in said space above said fibers, removing air from said space and permeating said space with vapor from said anhydrid, and heating the contents of said space until said fibers are acetylated.

2. The process of producing cellulose acetate which comprises introducing cellulosic material, liquid acetic anhydride and a catalyst into an enclosed vessel and maintaining said vessel at least partially evacuated until the cellulose has become acetylated.

3. The process of producing cellulose acetate which comprises introducing liquid acetic anhydride and cellulosic material which has been impregnated with an agent that promotes acetylation into an enclosed vessel and maintaining said vessel at least partially evacuated until the cellulose has become acetylated.

4. The process of producing cellulose acetate which comprises introducing cellulosic material, liquid acetic anhydride and a catalyst into an enclosed vessel, and heating the vessel and maintaining it at least partially evacuated until the cellulose has become acetylated.

5. The process of producing cellulose acetate which comprises introducing liquid acetic anhydride and cellulosic material which has been impregnated with an agent that promotes acetylation into an enclosed vessel, and heating the vessel and maintaining it at least partially evacuated until the cellulose has become acetylated.

Signed at Rochester, New York this 28 day of January 1928.

CARL R. NOLLER. 125